



US005925231A

# United States Patent [19]

Metzger

[11] Patent Number: 5,925,231

[45] Date of Patent: Jul. 20, 1999

[54] **METHOD FOR ELECTROPLATING ROTOGRAVURE CYLINDER USING ULTRASONIC ENERGY**[76] Inventor: **Hubert F. Metzger**, 1940 Lone Oak Cir. East, Brookfield, Wis. 53045[21] Appl. No.: **08/939,803**[22] Filed: **Sep. 30, 1997****Related U.S. Application Data**

[63] Continuation-in-part of application No. 08/854,879, May 21, 1997, abandoned, which is a continuation-in-part of application No. 08/755,488, Nov. 22, 1996, abandoned.

[51] **Int. Cl.<sup>6</sup>** ..... **C25D 5/02**; C25D 5/20; C25D 5/34[52] **U.S. Cl.** ..... **205/127**; 205/134; 205/137; 205/151; 205/205; 205/222[58] **Field of Search** ..... 204/199, 212, 204/222, 273; 205/127, 151, 205, 134, 137[56] **References Cited****U.S. PATENT DOCUMENTS**

- 2,702,260 2/1955 Massa ..... 204/273 X  
 3,351,539 11/1967 Branson .  
 3,647,646 3/1972 Tucker, et al. .  
 3,923,610 12/1975 Bergin et al. ..... 205/127 X  
 3,933,601 1/1976 Ishibashi et al. .  
 4,352,727 10/1982 Metzger .  
 4,503,769 3/1985 Andersen ..... 205/166 X  
 4,812,219 3/1989 Sattrup et al. ..... 205/223 X  
 4,830,758 5/1989 Bodine .  
 5,409,594 4/1995 Al-Jibory et al. .

**OTHER PUBLICATIONS**

H.E. Ricks, "Ultrasonics Improves, Shortens, and Simplifies Plating Operations," MPM (Mar. 1962) Best Available Copy.

W.D. Mogerman, "Ultrasonics in the Plating Industry," Plating (Aug. 1967) Best Available Copy.

Electroplating Engineering Handbook (Van Nostrand Reinhold Company, A. Kenneth Graham, ed. 1971) pp. 165-166, No month.

Ultrasonics General Information (printed from Internet on Nov. 14, 1996; dated Mar. 18, 1995).

Maurice O'Donoghue, The Ultrasonic Cleaning Process (printed from Internet on Nov. 14, 1996; dated Mar. 6, 1996).

J.R. Cox, "The Impact of Electromechanical Engraving Specifications on Streaking and Hazing," Gravure (Winter 1994) Best Available Copy No month.

R. Martin AG brochure entitled "Plating installations type B" (selected pages) (no date).

*Primary Examiner*—Donald R. Valentine  
*Attorney, Agent, or Firm*—Foley & Lardner

[57] **ABSTRACT**

An apparatus and method for electroplating and deplating a rotogravure cylinder out of a plating solution using ultrasonic energy is disclosed. The apparatus includes a plating tank adapted to rotatably maintain the cylinder and to contain a plating solution so that the cylinder is at least partially disposed into the plating solution. The apparatus also includes a mounting structure mountable within the tank partially on each side of and generally below the cylinder, along with a plurality of conductors at least partially disposed within the plating solution. A current source is electrically connected to the upper portions of the conductors and to the cylinder. An ultrasonic system to introduce wave energy into the plating solution includes at least one transducer element mountable within the tank and a power generator adapted to provide electrical energy to the transducer element. A holding tank having a circulating pump and heating and cooling elements for the plating solution may be provided. A method of preparing a rotogravure cylinder to be used in a printing operation is also disclosed.

**53 Claims, 17 Drawing Sheets**

FIG. 1





FIG. 2



FIG. 4



FIG. 5



FIG. 6







FIG. 10



FIG. 11

FIG. 12



FIG. 13



FIG. 14





FIG. 15



FIG. 16



FIG. 18





FIG. 18A



FIG. 25A





FIG. 23



FIG. 24



FIG. 25



FIG. 26





FIG. 27



FIG. 28



FIG. 29



FIG. 30

## METHOD FOR ELECTROPLATING ROTOGRAVURE CYLINDER USING ULTRASONIC ENERGY

### RELATED APPLICATIONS

This application is a continuation-in-part of application Ser. No. 08/854,879, titled "Rotogravure Cylinder Electroplating Apparatus Using Ultrasonic Energy" filed May 12, 1997, now abandoned, which is in turn a continuation-in-part of application Ser. No. 08/755,488, titled "Apparatus for Electroplating Rotogravure Cylinders Using Ultrasonic Energy" filed Nov. 22, 1996 now abandoned.

### FIELD OF THE INVENTION

The present invention relates to an apparatus and method for electroplating a rotogravure cylinder using ultrasonic energy.

### BACKGROUND OF THE INVENTION

In a conventional apparatus for the electroplating of a rotogravure printing cylinder, it is customary to rotate the cylinder (electrically charged as a cathode) in a tank filled with an electrolyte bath and copper bars or copper nuggets (electrically charged as an anode), as disclosed in U.S. Pat. No. 4,352,727 issued to Metzger, and incorporated by reference herein (wherein the copper nuggets are supported in a set of baskets made of titanium or of a plastic material and disposed around each side of the cylinder), or simply a plating solution.

In the arrangement shown in U.S. Pat. No. 4,352,727, the top edge of the respective baskets are disposed below the surface of the electrolyte bath so as to ensure free circulation of constantly refreshed (i.e. filtered) electrolytic fluid or solution. Electrolytic fluid is pumped into the tank from a manifold adjacent to the bottom of one of the baskets, in the direction of cylinder rotation. The top of the rotating cylinder to be plated is disposed slightly above the surface level of the electrolytic fluid so that a washing action occurs as the surface of the cylinder breaks across the surface of the electrolyte. Ions move from the copper bars or nuggets through the electrolytic fluid to the surface of the rotating cylinder during the plating process (or in the reverse direction in the deplating process). Where plating is done directly from a plating solution, ions move directly from the solution to the surface of the rotating cylinder.

Over time, refinements of this system have facilitated satisfactory control of the plating process, to achieve the desirable or necessary degree of consistent plating and uniformity in the plated surface of the cylinder. However, the complete process is comparatively slow, and extra polishing steps may be necessary after plating in order to produce a desirable uniform surface (e.g. roughness or grain structure) on the cylinder. According to the known arrangement, the overall efficiency of the process necessary to produce a suitably uniform plated surface on the cylinder can be adjusted either by reducing the current density, which increases the plating time but reduces the number or duration of additional polishing steps, or by increasing the current density, which reduces the plating time but increases the number or duration of additional polishing steps.

Furthermore, in the known arrangement, during operation, a copper sludge may tend to accumulate on and about the cylinder during the plating process, forming uneven and undesirable copper deposits, typically in areas of low current density (such as furthest apart from the copper

cylinder). A copper sludge may also build up between the contact surfaces of the titanium baskets or lead contacts. Moreover, other surfaces may become fouled with sludge and other matter.

Ultrasonic wave energy has been used successfully in surface cleaning applications. The long-known advantages in using ultrasonic energy in electroplating have also been described in such articles as "Ultrasonics in the Plating Industry", *Plating*, pp. 141-47 (August 1967), and "Ultrasonics Improves, Shortens and Simplifies Plating Operations," *MPM*, pp. 47-49 (March 1962), both of which are incorporated by reference herein. It has been learned that ultrasonic energy may advantageously be employed to improve the quality (e.g. uniformity and consistency of grain structure) of a plating process by providing for uniformity and efficiency of ion movement. In other applications, it has been found that copper can be plated onto a surface in a production system using ultrasonic energy at up to four times the rate ordinarily possible. It has also been found that the use of ultrasonic energy in an electroplating process provides an increase in both the anode and cathode current efficiency, and moreover, the practical benefit of faster plating with less hydrogen embrittlement (e.g. with less oxidation of the hydrogen on the plating and deplating surfaces).

Accordingly, it would be advantageous to have an apparatus configured to capitalize on the advantages of ultrasonic energy in the electroplating of a rotogravure cylinder. It would also be advantages to have an apparatus configured to use ultrasonic energy in the plating a rotogravure cylinder in order to obtain a more uniform and consistent grain structure on the plated surface of the cylinder through a more efficient process. It would further be advantageous to have a rotogravure cylinder plating apparatus employing ultrasonic energy to eliminate the build-up of copper (or other) sludge during the plating process.

### SUMMARY OF THE INVENTION

The present invention relates to an apparatus and method for electroplating and deplating a rotogravure cylinder out of a plating solution. The apparatus includes a plating tank adapted to rotatably maintain the cylinder and to contain a plating solution so that the cylinder is at least partially disposed into the plating solution, a mounting structure mountable within the tank partially on each side of and generally below the cylinder, and a plurality of conductors at least partially disposed within the plating solution. A current source is electrically connected to the conductors and to the cylinder. An ultrasonic system introduces wave energy into the plating solution. The ultrasonic system includes at least one transducer element mountable within the tank and a power generator adapted to provide electrical energy to the at least one transducer element.

The present invention also relates to a method of preparing a rotogravure cylinder to be used in a printing operation. The method includes the steps of pretreating the cylinder, plating the cylinder with a material while applying ultrasonic energy in a frequency range of 15 kHz to 40 kHz, and polishing the cylinder.

### DESCRIPTION OF THE DRAWINGS

FIG. 1 is a sectional elevation view of an electroplating apparatus for a rotogravure cylinder according to a preferred embodiment of the present invention.

FIG. 2 is a plan and cut-away view of the apparatus of FIG. 1.

FIG. 3 is a perspective view of the apparatus of FIG. 1 showing a basket system adapted to hold copper nuggets or the like.

FIG. 4 is a sectional elevation view of a plating tank of the apparatus of FIG. 1 showing a cylinder and the basket system.

FIG. 5 is a sectional elevation view of a lifter for the apparatus of FIG. 1.

FIG. 6 is a plan and cut-away view of a basket system for an electroplating apparatus according to an alternative embodiment.

FIG. 7 is a sectional elevation view of the apparatus of FIG. 6.

FIG. 8 is a sectional elevation view of a transducer assembly and a basket system for an electroplating apparatus according to an alternative embodiment.

FIG. 9 is a sectional elevation view of a transducer assembly and a basket system for an electroplating apparatus according to an alternative embodiment.

FIG. 10 is a sectional elevation view of a plating tank according to an alternative embodiment.

FIG. 11 is a schematic diagram of the ultrasonic transducer system.

FIG. 12 is a sectional elevation view of a plating tank according to an additional alternative embodiment configured to plate a rotogravure cylinder directly out of a plating solution.

FIG. 13 is a sectional and partial elevation view of a plating tank according to an additional alternative embodiment configured to plate a rotogravure cylinder directly out of a plating solution.

FIG. 14 is a sectional and partial elevation view of a plating tank according to an additional alternative embodiment.

FIG. 15 is a schematic elevation view of a conventional printing system.

FIG. 16 is a schematic perspective view of a system for engraving an image on a rotogravure cylinder.

FIG. 17 is a partially exploded perspective view of a plating tank (with a rotogravure cylinder) according to an alternative embodiment of the present invention.

FIGS. 18 and 18A are sectional end and elevation views of the plating tank of FIG. 17.

FIG. 19 is a sectional side and elevation view of the plating tank (with a rotogravure cylinder) of FIG. 17.

FIGS. 20 and 21 are plan views of exemplary arrangements of ultrasonic transducer elements within a plating tank according to alternative embodiments of the present invention.

FIG. 22 is a schematic sectional perspective view of a plating tank showing alternative arrangements of ultrasonic transducer elements.

FIG. 23 is a sectional side and elevation view of a plating tank (with a rotogravure cylinder) according to an alternative embodiment of the present invention.

FIG. 24 is a sectional end and elevation view of the plating tank of FIG. 23.

FIGS. 25 and 25A are sectional views of the mounting arrangement of an ultrasonic transducer element within the plating tank of FIGS. 18 and 18A.

FIG. 26 is a schematic view of an ultrasonic transducer element.

FIG. 27 is a schematic view of the grain structure of a rotogravure cylinder plated according to a conventional method.

FIG. 28 is a schematic view of the grain structure of the rotogravure cylinder plated according to a preferred embodiment of the present invention.

FIG. 29 is a photomicrograph of the surface of a rotogravure cylinder intended to correspond to FIG. 27.

FIG. 30 is a photomicrograph of the surface of a rotogravure cylinder intended to correspond to FIG. 28.

#### DETAILED DESCRIPTION OF THE PREFERRED EMBODIMENTS

Referring to FIGS. 1 through 4, a preferred embodiment of an apparatus for electroplating a rotogravure cylinder is shown. Apparatus 110 includes a plating tank 12 having side walls 12a and 12b, and walls 12d and 12e, and bottom 12c. Plating tank 12 as shown in FIG. 1 contains an electrolytic fluid (e.g. copper sulfate or the like in an appropriate solution) indicated by reference letter F at a level (indicated by reference letter L) regulated by the height of a weir 72 (e.g. the top of side wall 12b). A rotogravure cylinder 20 to be plated (or depleted) is rotatably supported at its ends (e.g. upon an extending central shaft) to be submerged into the electrolytic fluid approximately one-half to one-third of the cylinder diameter. Cylinder 20 is rotatably supported at its ends by bearings within a journal 22, in which it is rotatably driven by a suitable powering device (not shown). Cylinder 20, shown in the FIGURES as one of a standard size (e.g., having a diameter of approximately 800 to 1500 mm), is disposed in close proximity to a basket system 30; according to alternative embodiments cylinders of other diameters may be accommodated.

According to any preferred embodiment, the tank system and cylinder mounting and drive system are of a conventional arrangement known to those of ordinary skill in the art of rotogravure cylinder plating. In any preferred embodiment, apparatus 10 will include a basket system 30 having one or a plurality of basket compartments 32 formed by a series of side and internal dividing walls 31. Basket system 30 in any preferred embodiment be disposed into the electrolytic fluid below level 70 of the electrolytic fluid. To ensure complete and constant exchange of the electrolytic fluid, the exterior side walls of basket compartments 32 are maintained below level L, otherwise the flow of electrolytic fluid may stagnate between basket compartments 32 and cylinder 20 and may possibly cause overheating. The electrolytic fluid is itself of a composition known to those of ordinary skill in the art of electroplating, for example a solution of 220 to 250 gram/liter copper sulfate and 60 gram/liter sulfuric acid, to fill plating tank 12 to level L.

As shown in FIG. 2, basket compartments 32 of concavo-convex basket system 30 contain nuggets 34 of a metallic material such as copper to be plated onto (or depleted from) cylinder 20. Basket compartments 32 and partitioning walls 31 (shown in FIGS. 2 through 4) are formed from a suitable metallic material, typically titanium, or in an alternative embodiment, from a suitable plastic material such as polypropylene (as shown in FIG. 7). The arrangement of a basket system of this basic type is disclosed in U.S. Pat. No. 4,352,727 issued to Metzger, which is incorporated by reference. As shown, the basket compartments 32 of basket system 30 have concave walls that are disposed towards the surface of cylinder 20. According to a preferred embodiment, the distance between the anode surface of basket system 30 to the cathode surface of cylinder 20 is approximately 40 to 60 mm. According to any preferred embodiment of the present invention, basket system 30 does not encompass any substantial portion of the outer perimeter

of cylinder 20. (This relationship may vary in alternative embodiments which employ a basket system of a larger size relative to the cylinder.) As shown in FIGS. 3 and 4, basket system 30 is suspended from a pair of rails 40 extending along walls 12a and 12b of plating tank 12 by a series of hangers, shown as lead anodes 42. (Rails 40 are shown mounted from a reinforcing structure 41 in FIG. 1; according to an alternative embodiment, the ends of rails 40 may be supported by the tank ends or side walls.)

Lead anodes 42 provide electrical connection to rails 40 (e.g. bus bars), across basket system 30 and through basket compartments 32 in a manner so also to provide an electrical connection to electrically-conductive nuggets 34. (According to a preferred embodiment, high phosphor copper mini-nuggets, preferably 0.04 to 0.06 percent phosphor, are used.) As shown in FIGS. 3 and 4, nuggets 34 are contained in basket compartments 32 with overlaid plastic sheeting 36 (shown cut away in portions to reveal nuggets 34). (Plastic shield plates may be used when a cylinder of shorter length is plated so as to prevent over-plating at the cylinder ends.) According to this embodiment, lead anodes 42 (e.g. curved flat strips) serve as the structural supports (i.e. hangers) for basket system 30. Lead anodes 42 are mechanically fastened and electrically coupled to current-carrying rails 40 at junctions employing fasteners, shown as bolts 100. (According to a particularly preferred embodiment, the inner walls of basket compartments 32 have perforations and the outer walls of basket compartments 32 are solid, except for two rows of holes near their tops which enable the flow of plating solution through basket compartments 32.) Upper portions 42a of the lead anode strips 42 are dip coated to protect them from the electrolytic fluid; and lower portions 42b of lead anodes 42 are exposed and positioned within basket compartments 32 to maintain electrical contact with copper nuggets 34. In operation, the packing of copper nuggets 34 around and between lead anodes 42 and cylinder 20 to be plated protects lead anodes 42 against wear.

For plating the cylinder, the rails are connected to an anode side of a plating power supply (e.g. a current source of known design) and the cylinder is connected to a cathode side of the power supply; for de-plating, the anode-cathode connections are reversed. When the cylinder is printed out (i.e. after having been plated and etched), it is returned to the plating apparatus and deplated so as to return the copper to the nuggets.

Referring to FIGS. 1 through 4 (and also FIGS. 7 through 9), shown disposed lengthwise along the bottom surface of basket system 30 (e.g. bonded or securely mounted thereto) are ultrasonic transducer elements 50. Transducer elements 50 (shown as four elements 50a through 50d in FIGS. 1 through 4 and 7) are electrically coupled to a control system (shown schematically in FIG. 10) and are provided to introduce ultrasonic wave energy into plating tank 12. Transducer elements 50 can be of any variety known in the art. According to a particularly preferred embodiment, the transducer elements are designed to provide for operation in a frequency range of 15 to 30 KHz (cycles). In the exemplary embodiment shown in FIG. 1, two of the four transducer elements (e.g. outer transducer elements 50a and 50b) are configured and positioned in relation to basket system 30 as to assist with the plating process directly (e.g. to facilitate consistency of ion migration through the electrolytic fluid); the remaining two transducer elements (e.g. inner transducer elements 50c and 50d) are configured and positioned in relation to basket system 30 as to provide a cleaning function and maintain nuggets 34, cylinder 20 and other elements of

and about basket system 30 free of copper sludge and other fouling buildup.

As shown in FIG. 1, according to a preferred embodiment, the electrolytic fluid supply system functions as a closed circuit system. A supply of electrolytic fluid F is provided into plating tank 12 by at least one spray bar 62 (two are shown), which consists of a section of pipe or tube extending laterally along or near the bottom of plating tank 12. Each spray bar 62 has a series of apertures 62a along its length (as shown at least partially in FIG. 2) that provide for a constant and relatively well-dispersed flow of electrolytic fluid into plating tank 12 from a holding tank 14 (e.g. a reservoir). Holding tank 14 is formed of side walls 14a and 14b, a bottom 14d, a top 14c, and end walls 14d and e, and is disposed beneath plating tank 12 (e.g. top 14c of holding tank 14 matches bottom 12c of plating tank 12) so as to capture any flow of electrolytic fluid travelling over weir 72 in plating tank 12. (Electrolytic fluid F is maintained at its own level in holding tank 14.) Electrolytic fluid may build up heat and increase in temperature over time during the plating (or deplating) process and therefore holding tank 14 is equipped with a fluid cooling system 16 (e.g. a suitable heat exchanger for such fluid of a type known in the art). Likewise, electrolytic fluid may need to be heated from an ambient temperature to a higher temperature at the outset of the plating process and therefore holding tank 14 is also equipped with a fluid heating system 18 (e.g. a suitable heat exchanger for such fluid of a type known in the art). The temperature regulating system for the plating solution can be coupled to an automatic control system that operates from information obtained by temperature sensors in or near one or both tanks, and to control other parameters that may be monitored during the process, according to known arrangements.

During the entire electroplating process, the electrolytic fluid is constantly being filtered and the ultrasonic system is constantly running. Before the electroplating process begins, the ultrasonic system can be energized to provide for agitation of electrolytic fluid and for cleaning of the basket system (to eliminate metallic sludge) to provide for better contact between the metal nuggets and the titanium basket compartments and lead anodes (or the lead anodes themselves in an embodiment having plastic basket compartments).

A pair of supply pipes 60 feed spray bars 62 with a supply flow of electrolytic fluid. Supply pipes 60 each are coupled to a circulation pump 64 and a filter 66 (configured and operated according to a known arrangement). Circulation pumps 64 draw electrolytic fluid F from holding tank 14 into inlets 61 in each of supply pipes 60 and force it under pressure through filters 66 and into spray bars 62 where (having been filtered) it is reintroduced through apertures 62a into plating tank 12 for the electroplating process. Each of spray bars 62 extends along the bottom of plating tank 12, rising horizontally from holding tank 14 and turning at an elbow 68 to run horizontally along and beneath basket system 30. According to alternative embodiments, the apparatus could include one pump and filter coupled to either a single spray bar or a spray bar manifold system, or any other combination of elements that provide for the suitable supply of electrolytic fluid into the plating tank.

Referring to FIG. 2, a top (and broken away) view of basket system 30, plating tank 12 and holding tank 14, rails are shown disposed on a set of lifters (one is shown as hydraulic cylinder assembly 24 in FIG. 5), which allow the vertical position of the cylinder to be adjusted within plating tank 12 (in a set of end slots 26 in the end walls of the plating

tank that are adapted to form a leak-proof seal with the rotating cylinder assembly). The distance from the cylinder surface to the basket system, which is placed underneath the cylinder, may thereby be adjusted, for example, according to the diameter of the cylinder.

FIGS. 6 and 7 show an alternative embodiment of basket system 30a wherein basket compartments 32a are made of a plastic material (such as polypropylene according to a particularly preferred embodiment). Basket system 30a is supported by a combination of non-conducting weight-bearing support strips 43 (e.g. hangars) and conductive lead anodes 42a, both of which are bolted to rail 40. Support strips 43 cradle basket system 30a, passing under basket compartments 32a, to provide the primary supporting structure; lead anodes 42a pass through basket compartments and into electrical contact with nuggets 34a. Ultrasonic transducer elements 50a through 50d are also shown disposed beneath basket system 30 in FIG. 7. According to an alternative embodiment shown in FIG. 9, the apparatus employs a basket system 30 with two sets of basket compartments 32 disposed beneath the rotating cylinder. In the alternative embodiments shown in FIGS. 8 and 9, a single transducer element 50 is positioned beneath basket system 30.

Referring to FIG. 11, according to a preferred embodiment, the ultrasonic system includes an ultrasonic power generator 53 for transforming a commercial supply of electric power (e.g. typically provided at low frequency such as 60 Hz) to an ultrasonic frequency range (approximately 20 KHz), a transducer element 50 for converting the high frequency electrical energy provided by generator 53 into ultrasonic energy (i.e. acoustical energy) to be transmitted into and through the electrolytic fluid, and a low voltage direct current (DC) power supply 54 for powering generator 53 and transducer elements 50. As shown, ultrasonic transducer elements 50 are placed lengthwise under basket compartment 32 (or titanium tray) and have the surface from which the wave energy is transmitted oriented in a manner to promote an even exchanging of ions through electrolytic fluid F along the entire length of cylinder 20. Ultrasonic energy transmitted from the surface is also intended to agitate electrolytic fluid F and copper nuggets 34 thereby to "stir up" the copper sludge that tend to form (so that its constituents return to or tend to remain in the solution), according to phenomena employed in ultrasonic cleaning applications. In the preferred embodiment, the frequency and amplitude of the ultrasonic wave energy is maintained at a level (e.g. near 20 KHz) that tends to minimize the cavitation action that results from ultrasonic energy. Alternative embodiments, however, may operate at higher frequencies (e.g. above 20 KHz), where cavitation action tends to result, or may operate over a varying range of frequencies.

According to any preferred embodiment, the transducer elements efficiently convert electrical input energy from the generator into a mechanical (acoustical) output energy at the same (ultrasonic) frequency. The power generator is located apart from the plating tank, preferably shielded from the effects of the plating solution. The transducer elements can be generally of a ceramic or metallic material (or any other suitable material), preferably having a construction designed to withstand the effects of the plating solution in which they are immersed, and positioned to provide uniform energy (and thus uniform cavitation) throughout the basket system and rotogravure cylinder. (Exemplary transducer elements are described in the articles cited herein previously and incorporated by reference herein.) As shown in FIG. 9, a two basket system, ultrasonic energy (designated by reference

letter U) will pass between the basket compartments to cylinder (not shown). In an alternative embodiment shown in FIG. 10, transducer element 50 is mounted in a separate compartment formed between plating tank 12 and holding tank 14 that does not contain the plating solution; according to this embodiment the transducer element (or transducer elements) does not need to be designed to withstand the effects of the plating solution. Alternative embodiments may employ various arrangements of transducer elements to optimize plating (and deplating) performance in view of design and environmental factors (such as the ultrasonic energy intensity, flow conditions, sizes, shapes and attenuation of the tank, basket system, cylinder, etc.

The use of ultrasonic energy increases plating rates by 15 facilitating rapid replenishing of metal ions in the cathode film during electroplating. The ultrasonic energy is also very beneficial in removing absorbed gases (such as hydrogen) and soil from the electrolytic fluid and the surfaces of other elements during the electroplating process. According to any 20 particularly preferred embodiment, the transducer elements are arranged to provide ultrasonic energy at an intensity (e.g. frequency and amplitude) that provides for uniform and consistent agitation throughout the plating solution suitable for the particular arrangement of tank, cylinder and basket system. As contrasted to mechanical agitation, which may 25 tend to leave "dead spots" in the plating tank with where there is little if any agitation, ultrasonic agitation may readily be transmitted in a uniform manner (according to the orientation of the array of transducer elements).

Ultrasonic agitation according to a preferred embodiment will further provide the advantage of preventing gas streaking and burning at high current density areas on the cylinder without causing uneven or rough deposits. As a result, the 30 use of ultrasonic energy to introduce agitation into the plating tank produces a more uniform appearance and permits higher current density to be used without "burning" the highest current density areas of the cylinder like the edge of the cylinder. (Usually the critical area of burning or higher plating buildup is the edge of the cylinder.) (Ultrasonic energy also can be used in chrome tanks to increase the hardness of the chrome, to increase the grain structure of the chrome and to eliminate the microcracks in chrome.)

A further advantage of a preferred embodiment of the 35 plating apparatus using ultrasonic energy is that it expands the range of parameters for the plating process such as current density, temperature, solution composition and general cleanliness. The surface of a plated cylinder that used ultrasonic energy according to a preferred embodiment will 40 tend to have a much finer grain size and more uniform surface than a cylinder that used a conventional plating process. The plated surface hardness would typically increase (without any additive) by approximately 40 to 60 Vickers, evidencing a much finer grain structure. The use of ultrasonic energy in the plating process therefore allows a 45 minimum or no polishing of the cylinder while increasing the speed of deoxidizing of the nuggets and basket.

#### Additional Alternative Embodiments—Part 1

According to additional alternative embodiments, the 50 apparatus can be modified for plating or deplating a rotogravure cylinder with various metallic alloys or metals directly out of solution (i.e. without using metallic nuggets).

Apparatus 110 is shown in FIG. 12. Many of the same 55 elements of other embodiments described herein (e.g. apparatus 10) are present in apparatus 110. However, apparatus 110 (shown without any baskets or associated elements) is

adapted to plate cylinder 120 directly out of an electrolytic fluid a plating solution containing a plating metal or metal alloy in a plating solution indicated by reference letter F. According to this embodiment, cylinder 120 can be plated with any plating metal or metallic alloy. For example, cylinder 20a can be plated with chrome, zinc, nickel or other plating metal (including various alloys thereof) according to various processes known in the art.

Apparatus 110 includes a plating tank 112 of a type shown in FIG. 1 containing plating solution F at a level (indicated by reference letter L) regulated by the height of a weir 172. A rotogravure cylinder 120 to be plated (or deplated) is rotatably supported at its ends (e.g. upon an extending central shaft) to be submerged into the electrolytic fluid approximately one-half to one-third of the cylinder diameter. Cylinder 120 is rotatably supported at its ends by bearings within a journal, in which it is rotatably driven by a suitable powering device (not shown). Cylinder 120, shown in FIGS. 12 and 13 as one of a standard size (e.g., having a diameter of approximately 800 to 1500 mm); according to alternative embodiments cylinders of other diameters may be accommodated. According to any preferred alternative embodiment, the tank system and cylinder mounting and drive system are of a conventional arrangement known to those of ordinary skill in the art of rotogravure cylinder plating. The electrolytic fluid is itself of a composition known to those of ordinary skill in the art of electroplating.

Conductive curved anode strips are electrically connected to current carrying rails 144 and mounted in plating tank to make electrical contact with the plating solution (electrolytic fluid F). For plating the cylinder, the rails are connected to an anode side of a plating power supply (e.g. a current source of known design) and the cylinder is connected to a cathode side of the power supply; for de-plating, the anode-cathode connections are reversed. When the cylinder is printed out (i.e. after having been plated and etched), it is returned to the plating apparatus and deplated so as to return the plating metal to the solution. According to alternative embodiments, other conventional arrangements for effecting the electrical connections to the plating solution (electrolytic fluid) and the cylinder may be employed.

As shown in FIG. 2, a mounting structure 143 (oriented similarly to the anode strips) is mounted to (but not electrically connected to) rails 144. (Or it alternatively can be mounted to the walls of plating tank 112.) Disposed lengthwise along the bottom surface of mounting structure 143 (e.g. bonded or securely mounted thereto) are ultrasonic transducer elements 150. Transducer elements 150 (shown as four elements 150a through 150d) are electrically coupled to a control system (shown schematically in FIG. 10) and are provided to introduce ultrasonic wave energy into plating tank 112. Transducer elements 150 can be of a type disclosed herein or of any other suitable type known in the art. According to a particularly preferred embodiment, the transducer elements are designed to provide for operation in a frequency range of 15 to 30 KHz (cycles), although other ultrasonic frequency ranges (above 40 KHz and beyond) may be employed. Transducer elements 150 are configured and positioned to assist with the plating process (e.g. to facilitate consistency of ion migration through the electrolytic fluid), and to prevent any fouling buildup on the various elements of apparatus 110.

As shown in FIG. 12, according to a preferred alternative embodiment, the electrolytic fluid supply system functions as a closed circuit system. (As is apparent, this system is similar in structure and operation to other embodiments previously disclosed.) A supply of electrolytic fluid F is

provided into plating tank 112 by at least one spray bar 162 (two are shown), which consists of a section of pipe or tube extending laterally along or near the bottom of plating tank 112. Each spray bar 162 has a series of apertures along its length (similar to as shown at least partially in FIG. 2) that provide for a constant and relatively well-dispersed flow of electrolytic fluid into plating tank 112 from a holding tank 114 (e.g. a reservoir). A holding tank 114 is disposed beneath plating tank 112 so as to capture any flow of electrolytic fluid travelling over weir 172 in plating tank 112. (Electrolytic fluid F is maintained at its own level in holding tank 114.)

Electrolytic fluid may build up heat and increase in temperature over time during the plating (or deplating) process and therefore holding tank 114 is equipped with a fluid cooling system 116 (e.g. a suitable heat exchanger for such fluid of a type known in the art). Likewise, electrolytic fluid may need to be heated from an ambient temperature to a higher temperature at the outset of the plating process and therefore holding tank 114 is also equipped with a fluid heating system 118 (e.g. a suitable heat exchanger for such fluid of a type known in the art). The temperature regulating system for the plating solution can be coupled to an automatic control system that operates from information obtained by temperature sensors in or near one or both tanks, and to control other parameters that may be monitored during the process, according to known arrangements. Before the electroplating process begins, the ultrasonic system can be energized to provide for agitation of electrolytic fluid and for cleaning of the system to provide for better contact and plating performance.

A pair of supply pipes 160 feed spray bars 162 with a supply flow of electrolytic fluid F. Supply pipes 160 each are coupled to a circulation pump 164 (configured and operated according to a known arrangement that may or may not have a filter). Circulation pumps 164 draw electrolytic fluid F from holding tank 114 into inlets in each of supply pipes 160 and force it under pressure into spray bars 162 where it is reintroduced through apertures into plating tank 112 for the electroplating process. Each of spray bars 162 extends along the bottom of plating tank 112, rising horizontally from holding tank 114 and turning at an elbow to run horizontally along and beneath mounting structure 143. According to alternative embodiments, the apparatus could include one pump coupled to either a single spray bar or a spray bar manifold system, or any other combination of elements that provide for the suitable supply of electrolytic fluid into the plating tank.

An alternative embodiment is shown partially in FIG. 13 (certain elements of the apparatus are not shown), wherein the apparatus 210 employs an ultrasonic transducer element 250 that is cylindrical in shape (having a diameter of about 70 mm in a particularly preferred embodiment). Transducer element 250 is shown mounted within plating tank 212 by a mounting structure 243 (for example, as mounting structure 143 shown in FIG. 12). According to alternative embodiments, a mounting structure 243 integrated with the anode strips can be employed (compare FIG. 3). As shown, one transducer element 250 is mounted underneath rotating cylinder 220 by mounting structure 243 (at or near the level of the curved anode strips below cylinder 220 according to the preferred embodiment). One or more such transducer elements can be used according to alternative embodiments, for example, mounted in a spaced-apart arrangement along the mounting structure beneath cylinder 220. Underneath transducer element 250 is placed a reflector 260 having a highly polished reflective surface shown mounted to side walls of plating tank 212.

## 11

Reflector 260 is shown in the preferred embodiment as being of an integral unit having an arcuate shape, and extends substantially along the entire length of cylinder 220 (as does transducer element 250). Alternatively, the reflector can be provided with any other suitable shape (such as parabolic or flat or multi-faceted) or in segments. Transducer element 250 when energized will transmit wave energy (shown partially by reference letter U) in a substantially radial pattern through the plating solution, including toward cylinder 220 and against reflector 260 which will reflect the wave energy back to cylinder 220 and related structures (such as the anode strips). The direct and reflected ultrasonic wave energy is intended to keep the surfaces of the cylinder and related structures free of fouling buildup and to facilitate the plating process.

According to any preferred embodiment, ultrasonic wave energy can be used in the plating (and deplating) of various metals and metal alloys to the cylinder, as in chrome plating and also for plating alloys of zinc, nickel, etc. The ultrasonic system according any particularly preferred alternative embodiment will be capable of generating between two to six kilowatts of power; the system will provide ultrasonic energy at a frequency between 10 to 40 KHz (cycles per second).

As shown in FIG. 14, in alternative embodiments (similar to that shown in FIG. 13), other configurations of transducer elements (e.g. cylindrical in shape with a circular profile) can be employed. For example, four transducer elements 350a through 350d (shown in phantom lines) can be mounted in plating tank 312 at the sides of cylinder 220 (by a mounting structure fixed to the walls or base of the plating tank or some other suitable structure, not shown). According to an alternative embodiment, two transducer elements (e.g. 350b and 350d) can be used instead of four. (Transducer element 250 mounted by structure 243 and reflector 260 are also shown.) As is evident, a wide variety of transducer configurations can be made within the scope of the present invention, with any preferred embodiment including at least one transducer element positioned in or near the plating tank so that the beneficial effect of ultrasonic energy can be realized during the electroplating process. As FIG. 14 shows, such arrangements of transducer elements 350a through 350d (and 250) can also be employed in alternative embodiments used in connection with an electroplating apparatus that uses metal nuggets 334 maintained in basket compartments 332 (similar in arrangement to other embodiments described herein).

#### Additional Alternative Embodiments—Part 2

According to additional alternative embodiments, the apparatus can be modified for plating a rotogravure cylinder with various metallic alloys or metals (such as copper using metallic nuggets or chrome or zinc directly out of solution) to produce a uniform and consistent grain structure on the surface of the plated cylinder. Apparatus 410 is shown in FIGS. 17 through 26. Many of the same elements of other embodiments described herein (e.g. apparatus 10, etc.) are present in apparatus 410, or can be included in the apparatus according to various alternative embodiments.

In FIGS. 17 through 19, apparatus 410a is shown with basket compartments 432 and associated elements to plate a rotogravure cylinder 420 from copper nuggets 434 in a plating solution (indicated by reference letter F in other FIGURES). In FIGS. 23 and 24, apparatus 410b (shown without any baskets or associated elements) is adapted to plate cylinder 420 directly out of an electrolytic fluid (a

## 12

plating solution containing a plating metal or metal alloy in a plating solution indicated by reference letter F in other FIGURES). According to this embodiment, a cylinder 420 can be plated with any plating metal or metallic alloy. For example, the cylinder can be plated with chromium (chrome), zinc, nickel or other plating metal (including various alloys thereof) according to various processes known in the art.

Apparatus 410 includes a plating tank 412 of a type shown in FIG. 1 containing plating solution F at a level (indicated by reference letter L in other FIGURES). (The holding tank which can be positioned in any suitable location near the plating tank is not shown in these FIGURES.) Rotogravure cylinder 420 to be plated is rotatably supported at its ends (e.g. upon an extending central shaft) to be submerged into the electrolytic fluid approximately one-half to one-third of the cylinder diameter. Cylinder 420 is rotatably supported at its ends by bearings within a journal, in which it is rotatably driven by a suitable powering device (not shown). According to any preferred alternative embodiment, the tank system and cylinder mounting and drive system are of a conventional arrangement known to those of ordinary skill in the art of rotogravure cylinder plating. (Plating stations that may be adapted to incorporate the various embodiments of the present invention are commercially available, for example, from R. Martin AG of Terwil, Switzerland.) The electrolytic fluid is itself of a composition known to those of ordinary skill in the art of electroplating.

As shown in FIGS. 17 and 23, cylinder 420 has a cylindrical face surface 420a and opposing axial ends 420b (having a generally cylindrical shape). Ends 420b of cylinder 420 are installed into the apparatus according to a conventional arrangement to allow for axial rotation of the cylinder during the plating process. The cylinder assembly is shown generally in FIGS. 19 and 23. As shown schematically, each end 420b of cylinder 420 is mechanically coupled (e.g. using a chuck or like holding device) to an adapter 420c (also allowing for size differences in cylinders) which is retained within a bearing 420d (shown mounted to a bearing support 420e) for rotational movement about the axis of cylinder (e.g. imparted by a motor, not shown). Brushes 420f provide an electrical connection (i.e. as cathode) to cylinder 420.

According to an exemplary embodiment, the cylinder 45 includes a steel (e.g. 99 percent steel) base surface, as is conventional. Exemplary cylinders are commonly available (from commercial suppliers) in a variety of sizes, which can be plated according to the method of the present invention. Such cylinders after plating and engraving are used for 50 printing packaging or publications (e.g. magazines); exemplary cylinder surface diameters and lengths (i.e. surface area to be plated, engraved and printed out) will suit particular applications. Following the plating of the cylinder, the surface can be polished, then engraved with an image, 55 for example using engraving system 470 as shown schematically in FIG. 16, including a scanner 472, computer-based controller 474 and an engraver 476. Such systems are commercially available, for example, from Ohio Electronic Engravers, Inc. of Dayton, Ohio (Model No. M820). The 60 cylinder can be cleaned (and chrome-plated) and then printed out (according to processes known to those in the art who may review this disclosure), for example, onto a roll or web of paper using a printing system 480 (including cylinders 420) as shown schematically in FIG. 15. When use of the cylinder in the printing operation is completed, the image 65 is removed from the surface of the cylinder (e.g. stripped off if engraved on a Ballard shell or cut off if engraved on a base

copper layer). The cylinder can be cleaned and deoxidized, then replated (e.g. with base copper) and engraved for reuse. (Other materials may be similarly plated or engraved and printed on the cylinder by alternative embodiments, such as chrome or zinc.)

As has been described, the plating process is enhanced by the introduction of ultrasonic wave energy into the plating tank. An ultrasonic generator converts a supply of alternating current (AC) power (e.g. at 50 to 60 Hz) into a frequency corresponding to the frequency of the ultrasonic transducer system (oscillator); the usual frequency is between 15 or 20 kHz and 40 kHz. The energy to the transducer (from the generator or oscillator) is supplied by means of a protected connection (e.g. a cable) transmitting energy at the appropriate frequency. The transducer element converts the electrical energy into ultrasonic energy, which is introduced into the plating solution as vibration (at ultrasonic frequency). The vibration causes (within the plating solution) an effect called cavitation, producing bubbles in the solution which collapse upon contact with surfaces (such as the plated cylinder). The greater amount of ultrasonic wave energy introduced into the plating tank, the greater this effect.

Shown schematically in FIG. 22 are two types of ultrasonic transducer elements, cylindrical element 450x and rectangular element 450y. In preferred embodiments, as shown in FIGS. 19 and 23, an arrangement of cylindrical transducer elements 450 is used. The configuration of transducer element 450 (without sleeve) according to a particularly preferred embodiment is shown in FIG. 26. Transducer element 450 has end portions 450b and a central portion 450a; power is supplied at one of end portions 450b through an electrical connector 451 (shown as a cable which is coupled to the ultrasonic generator, not shown in FIG. 26). In an exemplary embodiment, the cylindrical transducer element has an overall length of approximately 1131 mm, a diameter of approximately 50 mm at its central portion and a diameter of approximately 70 mm at its end portions; such a transducer element provides approximately 1.5 kW of energy into the plating tank. (A transducer element of an overall length of approximately 1320 mm will provide approximately 2.0 kW; a transducer element of an overall length of 438 mm will provide approximately 0.6 kW.) In the preferred embodiment, each transducer element used in the apparatus is a high capacity (free-swinging) element, and provides a uniform sound field, enabling a high sound density. (Ultrasonic wave energy disperses radially from the axis of the transducer element, as shown in FIG. 13.) The transducer element is of a very compact (space-saving) design. As installed, it provides for easy replacement. According to particularly preferred embodiments, as installed, it is of a high durability (e.g. resistant to the effects of the plating solution). According to a particularly preferred embodiment, the system of ultrasonic transducer elements (and associated equipment) is provided by Tittgemeyer Engineering GmbH of Arnsberg, Germany. Ultrasonic transducer elements of varying shapes, sizes (lengths and diameters) and power, and associated ultrasonic generators are available from a variety of other sources and suppliers.

The apparatus can be constructed to accommodate rotogravure cylinders of a variety of sizes (e.g. smaller with a face length of 40 to 50 inches as used for packaging or larger, 72 to 148 inches as used for publications). The cylinder may have a standard diameter (of approximately 800 to 1500 mm) or, according to alternative embodiments, other diameters may be accommodated. As is evident from this disclosure, comparing FIGS. 18, 20 and 21, the ultrasonic transducer elements can readily be installed within the

plating tank in a suitable manner to introduce ultrasonic wave energy to facilitate the plating process. For example, two, three, or more ultrasonic transducer elements can be installed in a staggered or offset pattern to ensure coverage of (i.e. transmission of ultrasonic wave energy to) and along the entire length of the surface of the cylinder, as shown in FIGS. 20 and 21. According to an exemplary embodiment, each transducer element introduces about 1.5 to 2.0 KW of energy into the plating tank; if 6.0 KW of energy is to be introduced into the plating tank, three or four transducer elements can be installed, for example. For obtaining desirable results in the plating of smaller cylinders, two transducer elements may be used (3.0 to 4.0 kW); for longer cylinders, three or more transducer elements may be used (4.5 to 6.0 kW or more). According to a preferred embodiment, the amount of power to be applied by the transducer elements can be adjusted from 20 to 100 percent at the generator (oscillator) of the ultrasonic system. To optimize performance in a given application, other arrangements are possible using other transducer element combinations and power adjustment capability at the ultrasonic generator (e.g. 20 to 100 percent power).

The installation of the ultrasonic transducer elements of the apparatus according to a preferred embodiment is shown in FIGS. 18 and 24, and the other associated FIGURES. In FIGS. 18 and 18A, showing an apparatus adapted to plate copper from copper nuggets contained in basket compartments 432, transducer elements 450 are shown mounted to conductors shown as anode strips 442 (although another mounting structure could be used) which are coupled to current-carrying rails 444. In FIG. 24, showing an apparatus adapted to plate chrome or zinc or other metals directly from solution, a similar arrangement may be used (although a mounting structure distinct from the anode strips may be used); this apparatus includes an anode (mesh or expanded material) 443 positioned between transducer elements 450 and cylinder 420. The mounting arrangement includes supports 490 for the transducer elements. According to a preferred embodiment, support 490 may include an at least partially threaded rod 491 held at its base by two nuts 492 to anode strip 442 (or in other embodiments the mounting structure); a collar 494 is mounted to (threaded onto) rod 491. End 450b of transducer element 450 is fitted within collar 494 and secured therein by at least one retaining screw 495 (see FIG. 25 and 25A). (FIGS. 18A and 25A show an alternative embodiment of the mounting arrangement with a different collar fit.) The collar is preferably made of an electrically isolated plastic material; the transducer element is preferably covered with a sleeve 498 of an electrically isolated plastic material (such as a shrink-wrap tube of sufficient length). In each case, the objective is to prevent the build-up of plating material on the structures and withstand the effects of the plating solution. Other elements of the mounting arrangement are preferably treated with a resistant coating or made from a resistant material (or covered with electrical tape or the like) for isolation and also to withstand the effects of immersion in the plating solution. The supports can be provided in various shapes and lengths, in alternate locations (e.g. mounted to the wall or floor of the plating tank or to a supplemental structure), or with an adjustment capability, that allows the transducer elements to be positioned (at least vertically) in a functionally advantageous position within the plating tank. According to alternative embodiments, other mounting or fastening arrangements, for example, that withstand mechanical vibration and associated effects (e.g. loosening or fatigue), can be used.

FIGS. 20 and 21 show particular alternative arrangements of transducer elements intended to provide suitable "cover-

age" (i.e. generally uniform distribution) of ultrasonic wave energy along the length of the rotogravure cylinder (not shown), notwithstanding differences in cylinder length. In FIG. 20, a cylinder of intermediate length is accommodated; in FIG. 21, a longer cylinder is accommodated. Other arrangements can be provided to accomplish the goal of uniformity of distribution of ultrasonic wave energy to and along the cylinder. For example, transducer elements of a like type are available in other lengths, and may be used. In any preferred embodiment, however, the transducer elements should be arranged to provide for uniformity, notwithstanding the size or shape of the transducer elements. The amount of ultrasonic wave energy that is introduced into the plating tank to achieve the desired, consistent grain structure on the plated surface of the cylinder is roughly proportional to the plated surface area. For example, a 56-inch cylinder of approximately 10 inches in diameter uses approximately 3.0 kW of ultrasonic energy. Smaller surface areas require less energy; larger require more, roughly in this proportion. Ultrasonic wave energy requirements can be adapted to suit the application and will guide the arrangement of the transducer elements.

According to any preferred embodiment of the present invention, the rotogravure cylinder is provided with a plated surface having a consistent, even grain structure. Consistency of grain structure (and therefore of engraved "cells") within the plated surface of the rotogravure cylinder provides for higher quality of engraving and enhanced quality of rotogravure printing. Preferably, plating consistency is achieved in all dimensions, across and around the plated surface. The process of preparing the rotogravure cylinder for printing according to the various embodiments of the present invention is intended to provide the desired consistent grain structure for a variety of plated materials (i.e. copper, chrome, zinc, or the like). The process can be performed using apparatus as described in this disclosure or alternatively any other suitable apparatus adapted to practice the disclosed method.

In arranging or sequencing a series of steps (e.g. treatment) relating to the plating of the cylinder (i.e. the surface) according to preferred embodiments, various options are available. The cylinder is cleaned (a step that is regularly conducted after other method steps to ensure a quality plated surface for printing). A treatment of nickel or cyanide copper may be applied to the cylinder to facilitate plating. Alternatively base copper may be plated directly onto the cylinder. (According to the preferred embodiments of the present invention, copper may be plated directly onto the steel cylinder without the need for a special treatment.) According to exemplary embodiments, the base copper will have a thickness in a range between approximately 0.010 and 0.040 inches (though other thicknesses may be plated). If a Ballard shell is to be plated onto the cylinder, a separating solution will be applied to the base copper layer. The Ballard shell (if created) will preferably have a minimum thickness of approximately 0.003 inches or so (e.g. 0.0027 to over 0.004 inches).

According to the preferred embodiments, plating can be conducted in accordance with the same basic range of values of process parameters as for plating by convention methods (i.e. without using ultrasonic energy). The plating process according to the preferred embodiments is intended to produce a more uniform, consistent grain structure of the plated material as well as to speed the plating by allowing more energy (i.e. a higher current density on the plated surface) to be applied during plating without adverse effects. According to exemplary embodiments, copper can be plated

with a current density in a range of approximately 1 to 3 amperes per square inch (as compared with 0.8 to 1.2 amperes per square inch as an example for a typical conventional process); chrome can be plated with a current density in a range of approximately 5 to 12 amperes per square inch (as compared with 5 to 7 amperes per square inch as an example for a typical conventional process). As a result, in an exemplary embodiment, plating may be accomplished as much as 40 to 50 percent faster, or an increased thickness of plated material can be achieved in a given time period. For example, all other parameters being maintained constant, if a conventional system plates a Ballard shell of 0.0027 inches onto the cylinder in approximately 30 minutes without using ultrasonic energy, by using ultrasonic energy according to a preferred embodiment, after 30 minutes a Ballard shell of 0.004 inches in thickness would be plated onto the cylinder.

According to an exemplary embodiment for plating with copper (e.g. from copper nuggets), the plating solution is maintained at a temperature of approximately 25 to 35° C. (preferably 30 to 32° C.) with a concentration of 210 to 230 grams/liter of copper sulfate (preferably 220 grams/liter) and 50 to 70 grams/liter of sulfuric acid (preferably 60 grams/liter); ultrasonic energy (i.e. power) can be applied in a range of 1.5 to 6 kVA. According to a particularly preferred embodiment for plating with chrome (e.g. directly out of solution), the plating solution is maintained at a temperature of approximately 55 to 65° C. with an initial concentration of 120 to 250 grams/liter of chromic acid and 1.2 to 2.5 grams/liter of sulfuric acid; ultrasonic energy (i.e. power) can be applied in a range of 1.5 to 6.0 kVA. As is apparent to those of skill in the art who review this disclosure, the values of process parameters may be adjusted as necessary to provide a plated surface having desired characteristics. According to alternative embodiments, these ranges may be expanded further, using the advantages of ultrasonic energy.

In comparison to conventional methods (e.g. without using ultrasonic energy), the rotogravure cylinder plated according to any preferred embodiment of the present invention will provide a surface better suited for subsequent engraving and printing, as shown in FIGS. 28 and 30. The plated surface of the cylinder will be characterized by a hardness similar to that obtained by conventional methods, but the grain structure (i.e. size) will be more consistent across and along the surface (i.e. both around the circumference and along the axial length of the cylinder), by example (for copper plating) varying approximately 1 to 2 percent (with ultrasonic) in comparison to approximately 4 to 10 percent (without ultrasonic). (According to other exemplary embodiments, the plated surface hardness may increase 20 to 30 Vickers.)

The surface plated according to an embodiment of the present invention will exhibit an engraved cell structure 500 as shown in FIG. 28 (schematic diagram) and FIG. 30 55 (photomicrograph), with cell walls 502 of a generally consistent width and shape and relatively and substantially free of "burrs" or other undesirable deposits of material following the engraving process. By conventional methods, shown in FIGS. 27 and 29, the structure of cell 501 is somewhat less 60 consistent in form and dimension, as well as having material deposits 505 on or near walls 503 that may cause irregularities or defects during printing, see "The Impact of Electromechanical Engraving Specifications on Streaking and Hazing," Gravure (Winter 1994), which is incorporated by reference herein. Cells 500 of a consistent structure, as shown in FIGS. 28 and 30, with less distortion and less 65 damage during engraving, provide a surface on the cylinder

which can more efficiently be inked and cleaned and which is therefore more capable of printing a high quality image in the final product. When, as according to the present invention, such uniformity and consistency can be achieved across the length of the cylinder (not just in isolated portions of the surface), the overall printing quality is enhanced.

Although only a few exemplary embodiments of this invention have been described in detail above, those skilled in the art will readily appreciate that many modifications are possible in the exemplary embodiments (such as variations in sizes, shapes and proportions of the various elements, values of the process parameters, or use of materials) without materially departing from the novel teachings and advantages of this invention. Other sequences of method steps may be employed. Accordingly, all such modifications are intended to be included within the scope of the invention as defined in the following claims. In the claims, each means-plus-function clause is intended to cover the structures described herein as performing the recited function and not only structural equivalents but also equivalent structures.

Other substitutions, modifications, changes and omissions may be made in the design, operating conditions and arrangement of the preferred embodiments without departing from the spirit of the invention as expressed in the appended claims.

What is claimed is:

1. A method of preparing a rotogravure cylinder to be used for a printing operation so that when the cylinder is to be engraved a plated material on the cylinder provides a cell structure having a generally consistent shape and substantially free of irregularities, the method comprising:

(a) pretreating the cylinder;

(b) plating the cylinder with the plated material from a plating solution while applying ultrasonic energy from a transducer element arrangement having at least one transducer element installed beneath the cylinder in substantially parallel alignment with the cylinder to provide for coverage of ultrasonic energy along the cylinder so that the material is plated onto the cylinder with a substantially uniform grain structure; and

(c) polishing the cylinder;

wherein the step of plating the cylinder with the plated material is performed in an apparatus comprising a plating tank providing a floor being adapted to rotatably maintain the cylinder for rotation about a horizontal axis and to contain the plating solution so that the cylinder is at least partially disposed into the plating solution; a plurality of conductor having a first portion extending at least partially below the cylinder; a current source electrically connected to the conductors and to the cylinder; an ultrasonic system to introduce ultrasonic energy into the plating solution through the transducer element arrangement installed within the plating tank and a power generator adapted to provide electrical energy to the transducer element arrangement; and a mounting assembly, configured to mount the transducer element arrangement above the floor of the plating tank within the plating solution at a height no greater than the first portion of the plurality of conductors extending at least partially below the cylinder.

2. The method of claim 1 wherein the mounting assembly of the transducer element arrangement is at least partially integrated through the first portion of the plurality of conductors and the step of plating the cylinder while applying ultrasonic energy includes applying current from the first portion of the plurality of conductors.

3. The method of claim 1 wherein the transducer element arrangement includes at least one cylindrical transducer element mounted within the plating tank below the cylinder and the step of plating the cylinder while applying ultrasonic energy includes applying ultrasonic energy at least partially from the at least one cylindrical transducer element.

4. The method of claim 1 wherein the at least one transducer element is covered with an outer material resistant to the effects of the plating solution and the step of plating the cylinder while applying ultrasonic energy includes applying ultrasonic energy at least partially from the at least one transducer element through the outer material into the plating solution.

5. The method of claim 4 the outer material is electrically isolated from the current source and the step of plating the cylinder while applying ultrasonic energy includes applying ultrasonic energy from the at least one transducer through the electrically isolated outer material.

6. The method of claim 1 wherein the plated material is copper and the step of plating the cylinder is conducted at a current density in a range of approximately 1 to 3 amperes per square inch.

7. The method of claim 1 wherein the plated material is chrome and the step of plating the cylinder is conducted at a current density in a range of approximately 5 to 12 amperes per square inch.

8. The method of claim 1 further comprising the steps of:

(d) engraving the cylinder; and

(e) cleaning the cylinder.

9. The method of claim 8 further comprising the steps of:

(f) chrome plating the cylinder.

10. The method of claim 9 further comprising the steps of:

(g) polishing the cylinder.

11. The method of claim 1 further comprising the step of:

(h) printing from the cylinder.

12. The method of claim 11 further comprising the steps of:

(i) post-treating the cylinder; and

(j) cleaning the cylinder.

13. The method of claim 12 wherein the step of post-treating the cylinder includes the step of removing at least a portion of the plated material from the cylinder.

14. The method of claim 12 wherein the step of post-treating the cylinder includes the step of stripping the Ballard shell from the cylinder.

15. The method of claim 12 wherein the step of post-treating the cylinder includes the step of cutting at least a portion of plated material from the cylinder.

16. The method of claim 1 wherein the step of pretreating the cylinder includes the step of cleaning the cylinder.

17. The method of claim 16 wherein the step of pretreating the cylinder includes the step of plating the cylinder with a base copper.

18. The method of claim 1 wherein the step of pretreating the cylinder comprises the application of a separating solution to the cylinder and the step of plating the cylinder includes the plating of a Ballard shell onto the cylinder.

19. The method of claim 1 wherein the step of pretreating the cylinder includes the step of applying nickel to the cylinder.

20. The method of claim 1 wherein the step of pretreating the cylinder includes the steps of (a1) cleaning the cylinder and (a2) applying a cyanide copper treatment to the cylinder.

21. The method of claim 1 wherein the step of plating the cylinder with a plated material further comprises:

(b1) immersing the cylinder at least partially in the plating solution within the plating tank;

## 19

- (b2) maintaining the plating solution at a temperature of approximately 25 to 60 degrees Centigrade;
- (b3) applying a current density to the cylinder in a range of approximately 0.8 to 12 amperes per square inch;
- (b4) applying ultrasonic energy in a range of approximately 0.6 to 6 kW.

22. The method of claim 21 wherein the step of plating the cylinder with a plated material comprises plating the cylinder with copper.

23. The method of claim 21 wherein the step of plating the cylinder with a plated material comprises plating the cylinder with chrome.

24. The method of claim 21 wherein the step of plating the cylinder with a plated material comprises plating the cylinder with zinc.

25. The method of claim 1 further comprising the step of (d) engraving the cylinder, wherein the cell structure of the plated material on the engraved cylinder has walls of a substantially uniform width.

26. The method of claim 1 wherein the at least one transducer element is covered with a plastic material and the step of plating the cylinder while applying ultrasonic energy includes applying ultrasonic energy from the at least one transducer element.

27. The method of claim 1 wherein the step of plating the cylinder includes applying ultrasonic energy in a frequency range of 15 kHz to 40 kHz.

28. The method of claim 1 wherein the plurality of conductors includes a second portion and the step of plating the cylinder includes applying a current from the plurality of conductors into the plating solution with a current density in a range of approximately 1 to 12 amperes per square inch.

29. The method of claim 1 wherein the plurality of conductors is associated with at least one basket compartment and the step of plating the cylinder includes applying a current at least partially into the at least one basket compartment.

30. The method of claim 1 wherein the first portion of the plurality of conductors is associated with at least one basket compartment adapted to contain nuggets of the plated material and the step of plating the cylinder includes applying a current into the plating solution at least partially through the at least one basket compartment.

31. A method of preparing a rotogravure cylinder to be used for a printing operation so that when the cylinder is to be engraved a plated material on the cylinder is substantially free of irregularities, the method comprising:

- (a) pretreating the cylinder;
- (b) plating the cylinder with the plated material from a plating solution while applying ultrasonic energy from a transducer element arrangement having at least one transducer element covered at least partially with an outer material resistant to the effects of the plating solution installed beneath the cylinder in substantially parallel alignment with the cylinder to provide for coverage of ultrasonic energy along the cylinder; and
- (c) polishing the cylinder;

wherein the step of plating the cylinder with the plated material is performed in an apparatus comprising a plating tank providing a floor being adapted to rotatably maintain the cylinder for rotation about a horizontal axis and to contain the plating solution so that the cylinder is at least partially disposed into the plating solution; a plurality of conductors having a first portion extending at least partially below the cylinder; a current source electrically connected to the conductors and to

## 20

the cylinder; an ultrasonic system to introduce ultrasonic energy into the plating solution through the transducer element arrangement installed within the plating tank and a power generator adapted to provide electrical energy to the transducer element arrangement; and a mounting assembly configured to mount the transducer element arrangement above the floor of the plating tank within the plating solution at a height no greater than the first portion of the plurality of conductors extending at least partially below the cylinder.

32. The method of claim 31 wherein the mounting assembly of the transducer element arrangement is at least partially integrated through the first portion of the plurality of conductors and the step of plating the cylinder while applying ultrasonic energy includes applying ultrasonic energy from at least partially the transducer element arrangement at least partially across the first portion of the plurality of conductors.

33. The method of claim 31 wherein the transducer element arrangement includes a plurality of cylindrical transducer elements mounted within the plating tank below the cylinder and wherein the step of plating the cylinder while applying ultrasonic energy includes applying ultrasonic energy in a frequency range of 15 kHz to 40 kHz.

34. The method of claim 31 wherein the first portion of the plurality of conductors is a section of a generally arcuate-shaped anode and the step of plating the cylinder includes applying a current into the plating solution at least partially from the anode in a range of approximately 1 to 12 amperes per square inch.

35. The method of claim 31 further comprising the steps of:

- (d) engraving the cylinder; and
- (e) cleaning the cylinder.

36. The method of claim 35 further comprising the steps of:

- (f) chrome plating the cylinder.

37. The method of claim 36 further comprising the steps of:

- (g) polishing the cylinders.

38. The method of claim 37 further comprising the step of:

- (h) printing from the cylinder.

39. The method of claim 38 further comprising the steps of:

- (i) post-treating the cylinder; and
- (j) cleaning the cylinder.

40. The method of claim 39 wherein the step of post-treating the cylinder includes the step of removing at least a portion of the plated material from the cylinder.

41. The method of claim 39 wherein the step of post-treating the cylinder includes the step of cutting at least a portion of plated material from the cylinder.

42. The method of claim 31 wherein the step of pretreating the cylinder includes the step of cleaning the cylinders.

43. The method of claim 31 wherein the step of pretreating the cylinder includes the step of applying nickel to the cylinder.

44. The method of claim 31 wherein the step of pretreating the cylinder includes the steps of (a1) cleaning the cylinder and (a2) applying a cyanide copper treatment to the cylinder.

45. The method of claim 31 wherein the step of plating the cylinder with a plated material further comprises:

- (b1) immersing the cylinder at least partially in the plating solution within the plating tank;

**21**

- (b2) maintaining the plating solution at a temperature of approximately 25 to 60 degrees Centigrade;
- (b3) applying a current density to the cylinder in a range of approximately 0.8 to 12 amperes per square inch;
- (b4) applying ultrasonic energy in a range of approximately 0.6 to 6 kW.

**46.** The method of claim **31** wherein the step of plating the cylinder with a plated material comprises plating the cylinder with copper.

**47.** The method of claim **31** wherein the step of plating the cylinder with a plated material comprises plating the cylinder with chrome.

**48.** The method of claim **31** wherein the step of plating the cylinder with a plated material comprises plating the cylinder with zinc.

**49.** The method of claim **31** further comprising the step of (d) engraving the cylinder, wherein the cell structure of the plated material on the engraved cylinder has walls of a substantially uniform width.

**50.** The method of claim **31** wherein the outer material is electrically isolated from the current source and the step of

**22**

plating the cylinder while applying ultrasonic energy includes transmitting ultrasonic energy through the outer material into the plating solution.

**51.** The method of claim **31** wherein the plurality of conductors includes a second portion and the step of plating the cylinder includes applying a current into the plating solution from the plurality of conductors.

**52.** The method of claim **31** wherein the plurality of conductors is associated with at least one basket compartment and the step of plating the cylinder includes applying a current at least partially through the at least one basket compartment.

**53.** The method of claim **31** wherein the first portion of the plurality of conductors is associated with at least one basket compartment adapted to contain nuggets of the plated material and the step of plating the cylinder includes applying a current at least partially through the at least basket compartment.

20

\* \* \* \* \*